

## UNITED STATES PATENT OFFICE

CHARLES E. ALLEN, OF ROCHESTER, NEW YORK, ASSIGNOR TO EASTMAN KODAK COMPANY, OF ROCHESTER, NEW YORK, A CORPORATION OF NEW YORK

PROCESS FOR RECLAIMING FILM SCRAP WITH AN ALCOHOLIC SOLUTION OF SODIUM PEROXIDE

No Drawing. Application filed May 24, 1930. Serial No. 455,447.

This invention relates to the reclamation of dyed photographic film scrap having a base of a cellulosic derivative and more particularly to a process for reclaiming dyed photographic film scrap which has a base of cellulose nitrate.

For many photographic purposes, photographic films are tinted or colored with suitable dye which acts upon the film base or support to color it. The dye is usually applied to the film support upon the side opposite to which the light-sensitive silver halide emulsion is applied; the dye so applied does not normally penetrate more than a fraction 15 of a thousandth of an inch. Various methods have been employed for removing this dye from the film base in order that the film base may be re-employed for various purposes, such as the manufacture of new film, lacquers, 20 fabric coatings, etc.

Under normal practice, the silver halide emulsion is removed from the film by the use of hot water following which the dye is bleached and/or leached out of the film base.

Leaching with alcohol has been employed with success in some phases of film reclamation and bleaching of the film scrap is sometimes employed subsequent to the emulsion removal but prior to the leaching step.

It is among the objects of my invention to provide a simplified and efficient process which eliminates many of the steps and much of the cost and uncertainty of some of the prior known processes. It is a further object 30 to provide a process for reclaiming cellulosic derivative scrap. Other objects will be apparent herein.

I have found that dyed cellulose nitrate film base may be reclaimed in a very simplified manner, after the silver halide emulsion has been removed by hot water treatment from the cellulose nitrate base by subjecting the film scrap to the action of alcohol into which has been carefully stirred a small quantity of sodium peroxide. Such treatment is neither a leaching nor a bleaching process but is a single step method by which the surface of the cellulose nitrate film base is hydrolyzed and actually removed from the film. By so timing the treatment, the minimum amount

of surface thickness may be hydrolyzed so as just to remove that portion of the surface into which the film dye has penetrated or the amount of sodium peroxide stirred into the alcohol may be so limited that it is just slightly in excess of that necessary to hydrolyze the film base to the same depth as that to which the dye has penetrated.

As an example of my process, 2 to 30 grams of sodium peroxide may be slowly added with thorough stirring to one gallon of ethyl alcohol. The clear liquid is then decanted off and poured over approximately one pound of cellulose nitrate film scrap base from which the silver halide emulsion has previously been removed by hot water treatment. This treatment is carried on at approximately 90° to 120° F. and the duration of the treatment may be from 2 minutes to 1 hour depending somewhat upon the colors being treated and the depth to which the color has penetrated into the film base. The film is, of course, well agitated while being treated. The treatment should be continued only to the point at which all of the color is removed, at which time the alcoholic solution should be quickly drained away from the film scrap. This treatment is followed by subsequent washings with warm alcohol and finally by water. Instead of using regular commercial alcohol as a solvent for the sodium peroxide, mixtures of this alcohol in water may be used, the water being present in amounts as high as about 40% by weight of the total solvent mixture.

The sodium peroxide added to the ethyl alcohol does not accomplish my invention by virtue of any oxidizing action of the peroxide but by virtue of the fact that the sodium peroxide reacts with the water which is present in the alcohol employed to form caustic soda which goes into solution in the alcohol. The resulting alcohol solution of caustic hydrolyzes the surface of the film scrap base added to it. This hydrolysis is permitted to continue until it has penetrated to the same distance as the dye has penetrated. The hydrolyzed layer is soluble in the alcohol or alcohol and water mixture used with the sodium peroxide, and is consequently removed. Subsequent washings remove the remaining al-

kali and products of reaction so that clear film scrap results.

Merely because of the above specific example, I do not intend to be limited in the spirit or scope of my invention, inasmuch as it will be apparent that various alcohols may be employed, so long as the alcohol is not a solvent of the film base and will dissolve the caustic added thereto. Obviously other compounds may be added to the alcohol such, for instance, as potassium peroxide, etc., to produce a similar result, as well known to those skilled in the art. All of these modifications and equivalents are, of course, to be considered within the scope of the claims appended hereto.

What I claim as my invention and desire to be secured by Letters Patent of the United States is:

- 20 1. The process of removing dye from cellulose nitrate film scrap base which comprises treating the scrap with alcohol to which sodium peroxide has been added.
- 25 2. The process of removing dye from cellulose nitrate film scrap base which comprises removing the silver halide emulsion from the film base and then hydrolyzing the surface of the base with an alcohol solution to which sodium peroxide has been added.
- 30 Signed at Rochester, New York, this 20th day of May, 1930.

CHARLES E. ALLEN.

35

40

45

50

55

60